

Sept. 30, 1930.

L. L. LINICK

1,777,121

METHOD OF ELECTRODEPOSITION OF METALS AND ALLOYS

Filed Nov. 3, 1927

*Fig. 1*



*Fig. 2*

Inventor,  
Leslie Lloyd Linick  
Charles O. Stevens,  
his Atty.

## UNITED STATES PATENT OFFICE

LESLIE LLOYD LINICK, OF CHICAGO, ILLINOIS

## METHOD OF ELECTRODEPOSITION OF METALS AND ALLOYS

Application filed November 3, 1927. Serial No. 230,927.

This invention relates to a method of electro-deposition of metals and alloys, and among its objects are to produce a closer grained deposit than heretofore; to produce a faster deposit from a given solution without "burning" the cathode; to produce an equal or superior deposit from a weaker solution or from a given solution with a weaker current or lesser wattage; to produce a deposit of greater cohesion to its base; to produce a good deposit from a solution from which, otherwise, no electro deposit could be obtained, or only to a limited extent, or only erratic results could be obtained; to produce a good deposit of two or more metals in composition from solutions, which, otherwise, could not plate compositions or alloys; to obtain a deposit of precious metal directly upon aluminum; to obtain a deposit of precious and a base metal in composition directly upon aluminum and directly upon precious metal; to deposit metal upon plated ware. Other objects and advantages will occur in the course of this specification and with all of said objects and advantages in view, this invention consists in a method of electro-deposition of metals and alloys, with the use of an anode, in tube form, or contained in a glass tube or a tube made of other non-conducting insoluble material, and carrying and emitting an active gas under pressure to the surface or just below the surface of an electrolyte. It further consists in the method of electro-deposition of metals and alloys, wherein an active gas, under pressure, is introduced at or below the surface of an electrolyte for the purpose of electro plating. It further consists in the several novel features hereinafter fully set forth and particularly pointed out in the appended claims.

A simple form of apparatus for carrying on the method forming the subject matter of this specification is illustrated in the accompanying drawing in which—

Figure 1 is a diagrammatic view of the apparatus, partly in side elevation and partly in vertical section; and

Fig. 2 is an enlarged detail vertical sec-

tion through a certain anode supporting float employed in the apparatus.

Referring to said drawing, the reference character 3 designates a plating tank in which the electrolyte is contained. One or more reservoirs or gas tanks 4 are employed in which are separately contained active gases, such as hydrogen or oxygen, under pressure. Associated with each tank 4 is a pressure regulating valve 5 which is interposed in a main supply pipe 6 that leads from the gas tank 4, and said valve furnishes means whereby the pressure of the gas delivered into the solution in the plating tank may be regulated to obtain the desired result. A gauge 7 communicates with the pressure tank and indicates the pressure therein.

Interposed in the main supply pipe 6 beyond the pressure regulating valve 5 is a needle or other valve 8 for regulating the volume of gas delivered from the supply pipe. Adjacent said valve 8 is a gauge 9 for showing the pressure of the gas which is being used. Leading from the main supply pipe 6 is a flexible tube or supply pipe 10 which runs to a header 11 supported above the plating tank, and from said header lead individual flexible tubes or supply pipes 12 that are controlled by valves 13 interposed between the header and the individual flexible tubes 12.

The discharge ends of the flexible tubes 12 are supported directly above the surface of the plating solution in the plating tank 3, as, for instance, by floats 14 that rest upon the solution and are attached to the flexible tubes by bars 15 secured to the floats and having attaching nipples 16 fastened thereto, as best seen in Fig. 2. The flexible tubes 12 are slipped upon the ends of the attaching nipples 16, and in the lower ends of said attaching nipples are tubular anodes 17 preferably composed of platinum. The attaching nipples 16 are preferably formed of metal, and from said metal nipples extend the positive wires 18 of the plating circuit.

As many floats, gas supply tubes and anodes may be employed as is found best suited for the particular work at hand. As a preference, the floats with the anodes sup-

55

60

65

70

75

80

85

90

95

100

ported thereby are placed around the sides of the plating tank with the discharge orifice of the anodes touching the surface of the plating solution or barely immersed therein. A cathode 19, namely, the article or articles to be plated, is placed at or near the middle of the plating tank, and the negative wire 20 of the plating circuit leads to the cathode 19. The articles and individual flexible tubes may be suspended by wires or other similar means, as is well understood.

In carrying out the present method, any ordinary plating solution may be employed if desired and good results may be obtained with the use of the present method. The following solution has been found desirable for plating chromium:

|                   |                    |
|-------------------|--------------------|
| Water             | one-half gallon    |
| Chromic acid      | four ounces        |
| Pyrogallic acid   | eighteen grains    |
| Boric acid        | ten grains         |
| Chromium sulphate | ten grains         |
| Sugar             | twenty-five grains |

The above ingredients should be dissolved in hot water in the order given. When hydrogen gas is employed, the pressure of the hydrogen introduced into the plating tank should be approximately six ounces and the volume thereof should be sufficient to envelop the submerged parts of the anodes. Approximately from five to six volts of E. M. F. should be used at about one-tenth to one-eighth amperes per square inch of submerged cathode surface. The length of plating time should be from one minute to more, and the temperature of the plating solution should be about one-hundred-fifty to one-hundred-sixty degrees Fahrenheit. A solution containing chromium and platinum, for instance chromic acid and platinum chloride has been used to a great advantage.

The following is an example of said solution:

|                   |                 |
|-------------------|-----------------|
| Water             | one-half gallon |
| Chromic acid      | four ounces     |
| Platinum chloride | one-half ounce  |
| Ammonium oxalate  | one-half ounce  |
| Sodium phosphate  | one-half ounce  |
| Benzoic acid      | thirty grains   |
| Saccharose        | twenty grains   |
| Aluminum sulphate | twenty grains   |

The above ingredients should be dissolved in hot water in the order given. The pressure of the hydrogen introduced into the bath should be approximately four ounces and that of the oxygen should be approximately three ounces. The volume of the gases should be just sufficient to practically surround the submerged portions of the anodes. Approximately five volts of E. M. F. should be used at about one-fifteenth to one-tenth amperes per square inch of submerged cathode area.

The length of time for plating should be approximately two minutes or more, and the temperature of the bath should be about one-hundred-eighty to one-hundred-ninety degrees Fahrenheit.

I have discovered that an interrupted flow of electric current is beneficial to certain process of electro-plating, and that a pulsating direct current is similarly beneficial, producing better results and at a saving of time. With the use of a gas, under regulated pressure, flowing around the anode or anodes, I have been enabled to obtain an interrupted or pulsating effect on the electric current passing into the solution.

In the electrolyte formed by the solution, or just touching its surface, if desired, is placed a small anode or a number of small anodes, which may be of tubular or similar form, connected to a gas tank or other reservoir by a suitable conduit, which tank or reservoir contains gas, such as oxygen or hydrogen, under pressure, capable of being regulated by a suitable pressure regulating device and has control means, such as a needle valve, for regulating the flow or quantity of gas admitted to the solution. The anode or anodes are connected to the positive terminal of the plating line, and the cathode is connected to the negative terminal of the plating line as is well understood.

Specifically, a platinum hollow wire or tube of relatively small diameter and length may be used as an anode and this may be soldered to a copper tube. The tube may be connected by a flexible connection, such as a rubber hose, to the needle valve of a hydrogen or oxygen tank, provided with the usual pressure regulation means. The copper tube is connected by a copper wire to the positive terminal of the plating line. The hydrogen or oxygen (depending upon which gas is used) is allowed to flow to and through the platinum tube at a low pressure, for instance four ounces of pressure, with the platinum tube partly submerged in the solution or placed with its lower end in contact with it. The articles to be plated being placed in the solution and connected with the negative side of the plating line, the needle valve of the gas tank is opened and the gas permitted to discharge into the solution or on the surface thereof and the electric current is turned on for the required length of time (from a few seconds and upwards) to obtain the desired thickness of plate.

Instead of employing the platinum tube as the anode, the anode may be contained within a small glass tube and connected to the positive terminal of the plating line, and the glass tube connected by a suitable conduit, to the gas tank or reservoir. In either event, whether a single anode such as hydrogen gas, and in specified cases oxygen or other active gases, a plurality of anodes are used,

an active gas under regulated pressure are brought to or below the surface of the plating solution, which gas or gases envelop the anode to the surface of the solution, many times in excess of the natural gassing of an anode or electrode in an active plating solution.

When hydrogen and oxygen are both used they are brought to the solution in separate conduits and not as a mixture. Owing to the highly inflammable nature of these combined gases, it is advisable to install a suitable suction blower to carry off the escaping gases.

The anodes should be submerged alike and remain at a constant depth and in order to hold them at a constant depth, I use floats, in the center of each of which an anode is fastened, and I place the floats on the solution. The floats may be made of hard wood or other wood or of rubber tubular rings. Where any metal is used in the floats to support the anodes, such metal whether in the form of spokes or arms, should be placed above the surface of the solution. By supporting the anodes from the floats, the anodes are held in a vertical position, at right angles to the surface of the solution, whereby the escaping gas may completely envelop the anodes.

Comparing results of my method with other methods of electro-plating, I have found, that by the use of the hereinabove described process I am enabled to:

1. Obtain a closer grained deposit, which thus simplifies or eliminates subsequent polishing. This is of particular advantage with all plating, but especially in the plating of metals that are hard to polish, such as platinum, iridium, chromium, cobalt, tungsten, nickel and alloys of these metals.
2. Produce a faster deposit, from a given solution, without "burning" the cathode, or
3. Produce an equal or superior deposit from a weaker solution, or
4. Produce an equal or superior deposit from a given solution with a weaker current or a lesser wattage.
5. Produce a deposit of greater cohesion to its base.
6. Produce a good deposit from a solution from which, otherwise, no electro-deposit could be obtained.
7. Produce a good deposit from a solution from which, otherwise, electro-deposition could be obtained only to a limited extent.
8. Produce a good deposit from a solution from which, otherwise, only erratic results are obtained.
9. Produce a good deposit of two or more metals, in composition, from solutions, which, otherwise, could not plate compositions or alloys.
10. Obtain a deposit of precious metal directly upon aluminum.

By experiment, I have found that the

pressure of gas or gases must be proportioned to the volume of the cathode, to the rate of the current used and to the displacement of the anode. Thus, with a bulky article, I use a greater anode surface, represented by more 70 anode tubes in number, and a correspondingly greater pressure of the gases employed, which in turn regulates the flow of current independent of rheostat regulation. By the use of several anodes, barely submerged and emitting hydrogen from one and oxygen from the other, the deposition is greatly improved in many cases. I have used these gases and others, singly and together, with one or more anodes, soluble and otherwise 80 for electro-deposition purposes and have obtained the results mentioned in this specification.

I find it advisable where hydrogen and oxygen are both employed to use an excess 85 of hydrogen with precious metals in general, and with chromium and cobalt. With most other metals, I use an excess of oxygen. I have had good results with cobalt, platinum, chromium and iridium by the sole use of 90 hydrogen.

Using my process, I have successfully plated silver and other metals in varying thicknesses upon negative and positive films and prints, including motion-picture films 95 and stereopticon slides; also directly upon non-metallic objects, such as plant-leaves, insects, flowers, corals, shells, cameos and pearls. The electro-deposition of metals and alloys on the latter mentioned articles is of 100 value for the following reason:

A piece of jewelry set with coral, cameos, pearls, shell, or other organic substances cannot be plated in a solution which attacks these organic substances, such as chromic acid solutions. A piece of jewelry plated with chromium cannot be set after plating, as the plate is too hard or brittle. However, by first plating such organic substances with a metal upon which chromium cannot be plated in an ordinary solution, such organic substances can then be set into pieces of jewelry and the piece can be chromium plated in an ordinary solution, and then the plate on the inset part removed with an acid that will dissolve its 115 plated coating without attacking either the chromium plate or the set part.

The results obtained by my present process I ascribe to: (a) The interruption by means of an active gas of the flow of the electric current within a plating solution. This interruption may be complete or incomplete, passing continuously or intermittently. (b) The chemical action, the electrolytic action and the mechanical action of the gas or gases upon 120 the solution, the anode and the cathode or either of these.

I desire it to be understood that the expression "gas under pressure" in this specification and in the following claims means a gas not 130

produced within the solution or electrolyte, but brought to the solution or electrolyte from without by means of a conduit or similar gas conveying medium.

- 5 In general, the gas pressure should be sufficient to allow the gas to flow, while the volume should be great enough to almost completely envelope the submerged sections of the anodes. Platinum, tungsten, lead, steel or carbon anodes may be used with about equally good results. In the plating of cadmium, nickel, zinc, copper, silver, palladium and gold, soluble anodes of the corresponding metals may be used in the manner above explained. Anodes should be well distributed along the walls of the tank, their combined submerged area being about one-half of that usually required for the particular metal in question. In plating with the described formulas, I have successfully used an area about one-quarter that of the cathode surface.

10 I claim as new, and desire to secure by Letters Patent:

1. The method of electro-deposition of metals and alloys, which consists in conveying hydrogen gas and emitting the gas, under pressure, in contact with an electrolyte while an electric current is passed through the electrolyte.
2. The method of electro-deposition of metals and alloys, which consists in conveying and emitting hydrogen gas, under regulated pressure, below the surface of an electrolyte while an electric current is passed through the electrolyte.
3. The method of electro-deposition of metals and alloys, which consists in emitting hydrogen gas, under regulated pressure, from an insoluble tubular anode in contact with an electrolyte, while an electric current is passed from said anode through the electrolyte.
4. The method of electro-deposition of metals and alloys, which consists in surrounding an anode with hydrogen gas under regulated pressure, while partly submerged in an electrolyte.
5. The method of electro-deposition of metals and alloys, which consists in surrounding an anode with hydrogen under pressure, while partly submerged in an electrolyte.
6. The method of electro-deposition of metals and alloys which consists in conveying and emitting gas under a regulatable pressure immediately below the surface of an electrolyte while an electric current is passed through the electrolyte.

LESLIE LLOYD LINICK.